

Dec. 18, 1956

H. A. SECRIST

2,774,127

TEXTILE SHEET MATERIAL

Filed Oct. 24, 1950



INVENTOR.  
HORACE A. SECRIST  
BY H. L. KIRKPATRICK  
ATTORNEY

1

2,774,127

## TEXTILE SHEET MATERIAL

Horace A. Secrist, Dedham, Mass., assignor to The Kendall Company, Boston, Mass., a corporation of Massachusetts

Application October 24, 1950, Serial No. 191,933

5 Claims. (Cl. 28—79)

This invention relates to conformable textile sheet materials which consist in part of fibers which have been spun into yarns and in part of integrated unspun fiber masses.

In the past composite structures of spun and unspun fibers have been produced by adhesively joining woven fabrics to loosely associated fiber masses or to adhesively bonded non-woven fibrous sheets. The adhesive connections have consisted of fiber-to-fiber and fiber-to-yarn bonds created by saturating or impregnating the assembly with elastomeric or other resinous substances or by activating potentially adhesive fibers contained in the structure. In some instances woven bases and fibrous bodies have been loosely connected by mechanical techniques. Because of the low degree of frictional entanglement, however, the fiber anchorage is usually so poor that these structures have unsatisfactory abrasion or delamination resistance unless they are further united by positive adhesive bonding between the fibers and the yarns.

If the composite fabrics have been saturated or impregnated with cementitious substances, the porosity of the structure as a whole is commonly reduced and its absorbency and softness are usually greatly diminished. In those cases where potentially adhesive fibers have been used as bonding agents, the pressure usually employed during unification of the assembly mats down the fibers causing a similar loss in bulk, softness and porosity. In such prior structures, the dominant characteristics of the woven base fabric largely control the physical properties of the product because the low extensibility of the woven fabric and its adhesive bonding to the unspun fibers minimize freedom of fiber movement.

It is the primary object of this invention to provide a unital structure of spun and unspun cotton fibres which, in itself, has sufficient integrity to obviate the necessity for adhesive binder materials.

It is a further object of this invention to provide an integrated structure of spun and unspun cotton fibers which has extensibility (much or little as may be desired), exceptional stress distribution capacity, conformability, elastic return, and substantial tensile strength when the limit of its normal extensibility is approached.

It is a still further object of this invention to provide a soft, flexible sheet material of spun cotton fibres and self-integrated masses of unspun cotton fibres, the unspun fibers being arranged at one or more surfaces of the sheet material.

I accomplish these objects, and others, by supplying a novel unital fabric comprising spun and unspun fibers, the fabric being characterized by frictional entanglement and interlocking of the unspun fibers with each other and with the spun fibers, individually, collectively, or both, as a result of artificially induced kinks, bends, twists and curls in a portion at least of the unspun fibers, with or without the same in the spun fibers. In my preferred structures the yarns exhibit random kinks, bends, loops and twists, further enhancing the integration of the spun and unspun fibers but, in various useful products of sub-

2

stantial integrity, yarns may be practically straight or exhibit only a slight crimp.

These and other characteristics of my invention will be more readily appreciated from the following description of several embodiments thereof selected for the purpose of illustration and shown in the accompanying drawings, in which:

Figure 1 is a plan view of a section of fabric in accordance with one embodiment of my invention.

10 Figure 2 is a cross section along line 2—2 of Figure 1.

Figure 3 is a plan view of another fabric according to my invention, one corner of the fabric being sectioned in the plane of the yarns, and the upper layer of unspun fibers being rolled back upon itself.

15 Figure 4 is a cross section along line 4—4 of Figure 3.

Figure 5 is a plan view of a section of a fabric in accordance with another embodiment of my invention.

20 Figure 6 is a cross section along line 6—6 of Figure 5.

Referring to the drawings, the fabric comprises a composite of spun fibers or yarns 10 and unspun fibers 12. The spun fibers 10 may be randomly disposed as shown in Figures 1 and 2, or may be woven into fabrics as shown in Figures 3 and 4, or may be knitted as shown in Figures 5 and 6, or may be netted or otherwise disposed. The spun fibers 10 are in commingled relationship with the unspun fibers 12. The yarns or unspun fibers 12 are mutually integrated and are in apposition with the spun fibers 10, as a result of the kinks, bends, twists and curls of unspun fibers 12.

25 Substantial fiber freedom is maintained in the association of yarns and unspun fibers in the basic fabric because no bonding agents are required to lock the fibers into any fixed orientation or arrangement; however, the frictional engagement and entanglement of the unspun fibers with each other and with the spun fibers is substantially continuous and uniform throughout the sheet and contributes unusual tensile characteristics to the sheet material. The preferred products of this invention possess conformability and extensibility due, it is thought, to the capacity of the curled unspun fibers to straighten, extend, slip past each other and assume new positions of entanglement coupled with the stress distribution action of the spun fibers. In general, typical novel sheet materials of my invention may be extended 25% in either direction without any appreciable destruction of integrity, although, in some instances, depending on the yarn construction and conditions of treatment, the extensibility is considerably less, while in my preferred structures the extensibility is generally 75% or better and elongations at break of as high as 150% have been noted. Unlike conventional

30 materials of high extensibility which tend to rupture with only slight increases in stress as their stretch limits are approached, many or most of my products exhibit a high ultimate strength in one or more directions when the limit of ready deformation is reached, and substantial increases in deformation stresses produce only slight additional elongations.

35 When my preferred sheet materials are subjected to tension along either of their axes, the structures display a relatively high initial resistance to deformation, and thereafter the elongation is relatively large for small load increments until the modulus increases to a value which remains substantially constant up to the break point of the material. The smooth, continuous shape of typical stress-strain curves prior to the inception of failure is an indication of the striking interaction and cooperation of the spun and unspun fibers when the structure is subjected to deformation stresses and evidences the integral character of my novel fabrics. Further, the tendency of both types of fibers to return to their original contracted configurations on the removal of applied stresses provides my fabrics with a substantial degree of elastic return.

The strength, elastic conformability and capacity for stress distribution of my novel products in combination with their capacity to receive large quantities of saturants or impregnants adapts them for use as base materials in the manufacture of plastic laminates, artificial leather, shoe stiffeners and the like.

For example, when base materials for deep drawn plastic laminates are forced into a mold by the pressure of a molding die, severe local stresses are developed in the material at the edges, corners and planar intersections of the mold. Even woven fabrics of relatively high tensile strength frequently rupture under these conditions because they lack the extensibility and conformability for three-dimensional yield without failure. Fibrous bats and other non-woven fibrous sheet materials which are frequently used for this purpose, although they may possess the necessary extensibility and conformability to yield without rupture, lack the stress-distribution capacity for uniform, smooth deformation. As a result, even if complete failure of such non-woven base materials is avoided, the finished deep-drawn products have pronounced thick and thin spots, are unsightly in appearance and susceptible to failure under further stresses.

In my novel sheet materials, including a layer or layers of yarns, the yarns, so to speak, act as conductors of stress away from stressed local areas so that when my products are subjected to tension and/or two or three-dimensional deformation stresses, the load is distributed throughout a larger zone of the structures rather than carried by single fibers or local groups of fibers, and the occurrence of thick and thin spots is minimized.

Because the natural softness and absorbency of the cotton fibers need not be destroyed or inhibited by the addition of bonding agents, many of my structures have general utility in the medical and surgical field as dressing and bandaging materials, particularly when appreciable strength and limited elasticity are desired, as in the wrapping of sprained limbs or fractured ribs. Furthermore, the high degree of fiber association provides a dressing which is substantially resistant to linting, and the pure cellulose content of my preferred structures permits standard sterilization techniques and avoids possible contamination of wounds with non-cellulosic material which may be of an irritating or toxic character. As polishing cloths or as applicators for wax, shoe polish, cleaning compounds and the like, the products of this invention are highly satisfactory. Their ready conformability enables them to be drawn about polishing blocks or plates without fabric rupture and the fiber absorbency and the high percentage of voids in the structures permits the introduction of large amounts of polishing or cleaning mediums.

Since my products consist entirely, or mainly, of cellulose, they are particularly useful as industrial filters or in other similar applications where a high resistance to the action of a wide variety of inorganic or organic solvents is required. Fibrous materials which contain binder materials or which have been reinforced with or laminated to woven fabrics by means of added binding agents are restricted in their usefulness for filtering purposes because of the danger that the liquid to be filtered may dissolve the binder material, thereby weakening the filter structure and contaminating the liquid.

Preferably, I prepare the novel fabrics of my invention in the following manner. One or more unspun cotton fiber layers, preferably carded or garnetted webs, placed in intimate contact with one or more layers of spun cotton fibers, are subjected to treatment with alkaline liquids having a substantial swelling action on cellulose in such a manner as to permit substantially unrestrained or controlled shrinkage of the structure, depending on the characteristics desired in the final product. The integrated assembly is then washed to remove the swelling agent and dried. The preferred treating chemical of the process is an aqueous solution of caustic alkali such as sodium, potassium, or lithium hydroxide, but other basic cellulose

swelling agents may be employed, such as solutions of sodium zincate, quaternary ammonium bases such as benzyl trimethyl ammonium hydroxide and the like.

An apparatus which may be employed in the manufacture of my products is disclosed and more fully described in my copending application, Serial No. 151,512, filed March 23, 1950, now Patent No. 2,688,864.

Using aqueous sodium hydroxide solutions satisfactory results have been obtained with solution concentrations of at least 8% and less than 30% NaOH at temperatures from just above the freezing point of the solution to +25° C. Temperature and concentration are mutually dependent variables, and the selection of a particular value for one may fix the operating range of the other. Preferably and for best results such solutions are used in concentration of at least 10% and less than 18% NaOH at temperatures from -10° C. to +15° C. Other reagents may be employed at corresponding effective strengths and temperatures.

The maximum felting, contractive effects of the chemical are realized in a short time, normally in 1/2 to 3 minutes, and the sheet material is then removed from the vat and treated to remove the chemical, preferably promptly as over-long exposure to the chemical, especially in air, may produce secondary changes in the fibers which may give undesirable results.

The chemical solution is washed from the shrunken sheet material preferably by flowing a large quantity of water through it while it is carried on a moving screen or like structure through which the liquid drains. Preferably, although not necessarily, the alkaline residue is then neutralized in acid or other suitable agent, such as acetic acid or sodium bicarbonate, and the sheet material is again washed. The fibrous sheet material washed free of treating chemicals is finally dried to complete the process.

If high residual stretchability is undesirable or unnecessary, as for example in those instances in which my sheet materials are to be used as polishing or wiping cloths, integral products of limited extensibility in one or both directions, may be manufactured either by restricting the shrink of the assembly by varying the yarn construction or the treating conditions, or by wet-stretching the caustic-treated sheet material and drying. These variations in the production process afford commercial economy because of the increased yardage obtained from the same raw material.

The preferred spun fiber constituent of my invention is an open-mesh woven fabric usually disposed in uniform layer form coextensive with the unspun fiber constituent during integration therewith. Similarly, it may consist of a knitted or netted fabric disposed in like manner or, it may take the form of yarns laid in the warp direction only, in the filling direction only or otherwise positioned with the unspun fiber constituent.

In structures embodying a knitted yarn layer or layers, the high degree of freedom of the knitted yarns promotes particularly good interaction between the yarns and unspun fibers during my treatment but also deprives these structures of the sharply defined limit of extensibility which is desirable for some purposes.

Either the yarns or the unspun fibers may predominate at one surface or at both surfaces of the structures and various multiple structures may be manufactured depending on the number and orientation of the spun and unspun elements. Figures 3 and 4 show the unspun fibers 12 predominately at both surfaces of the fabric, and Figures 5 and 6 show the spun fibers or yarns 10 predominately at one surface of the fabric. In those structures where yarn arrangements other than woven or knitted fabrics are employed it may be preferred that the spun fibers be buried in the interior of the material for the sake of more uniform appearance, and/or surface characteristics, integrity, etc.

In any case, it is emphasized that the novel fabrics

of the present invention are unital structures in which the constituent parts are mutually integrated by the artificially-induced interlocking fiber configurations.

When the assembly is treated with caustic, the unspun fibers writhe, curl, twist and loop in all three dimensions, entangling themselves with each other and with the spun fibers to which they are in apposition, the unspun fibers in some cases penetrating the interstitial yarn spaces and looping around the yarns, and the frictional engagement of the two types of fibers being further increased in my preferred structures by the contractions and distortions of the yarns and the entrapment of unspun fibers between kinks and bends of the yarns.

I prefer open-mesh fabrics as the sun-fiber constituent of my structures because they permit high area contractions and maximum integration with the unspun elements. However, useful structures of integrity sufficient for many useful purposes may incorporate closely meshed yarns. If the yarns are arranged otherwise than by weaving or knitting, the same general considerations apply.

In the manufacture of my products I have found it commercially expedient to employ unspun fiber layers ranging in weight from five grams per square yard to 150 grams per square yard. In order to attain various objects of this invention, it is necessary only that spun fibers be present in significant amounts.

While the products of this invention are prepared by chemically treating spun and unspun cotton fibers, and such products are primarily dependent for their structural integrity on the presence of interlocking cotton fibers, it is possible to prepare many useful articles in which other fibers may be dispersed in minor proportion provided that they do not seriously interfere with the interlocking of the cotton fibers. These additive fibers may be cellulosic or non-cellulosic, thermoplastic, natural or synthetic fibers, such as kapok, wool, silk, vinyon, nylon, and regenerated cellulose. If desired, rubber-cored yarns may be employed.

In the preparation of my unspun fibrous web constituents I usually employ cotton fibers of sufficient length to be handled conveniently on textile machinery such as cards or garnets. However, the fiber length is not critical provided that the fibers can be assembled pneumatically or otherwise into webs sufficiently coherent to be processed by my caustic treatment and the fiber length-to-diameter ratio is sufficiently large to permit adequate entanglement of the fibers with each other and with the yarns.

To illustrate further suitable preferred practice of the process of my invention and production of various novel fabrics thereof, the following examples are given:

*Example 1*

Webs of cotton fibers from two cards were superposed to form a fibrous sheet weighing 15 grams per square yard. Between two such sheets was placed a coextensive layer of 14 x 10 open mesh, bleached cotton fabric woven of 30's and 40's yarns in the warp and filling respectively. The assembly was lightly pressed by passing it through nip rolls under a pressure of about 10 pounds per inch of roller width and then treated in a 16% solution of sodium hydroxide at a temperature of -2° C. After a treating period of 35 seconds the structure was removed from the bath by means of a moving screen, rinsed with water, neutralized with acetic acid, again washed, and finally dried on dry cans. An area shrink of the order of 85% was noted. As a variation of this example, the woven fabric might have been at both surfaces with the fibrous sheet therebetween.

*Example 2*

A ply from a 45 grams per square yard header roll of superposed webs of bleached, carded cotton fibers was lightly pressed to a layer of 18 x 12 cotton gauze and the assembly treated in 18% caustic at 10° C. After the

integrated sheet material was washed with water, neutralized with acetic acid, rewashed with water and dried on a steam can, an area shrink of approximately 75% was noted.

*Example 3*

Grey knitcloth, having 6 wales and 8 courses per inch of 29's cotton yarns, was boiled and bleached. A layer of this cloth was lightly pressed to a piece of the same dimensions from a header roll of bleached, carded cotton, and the assembly treated in a 16% solution of NaOH at -2° C. The area shrink of the material, measured after washing and drying, was 85%.

*Example 4*

A layer of cotton from a header roll and a coextensive piece of 14 x 10 raw cotton fabric (of 30's and 40's yarns having normal twist) in the loom state, i. e. with sizing on the warp yarns, were lightly pressed together and dropped into a tank containing 11.8% NaOH at 0° C. and a small amount of a suitable wetting agent. The resulting area shrink, after washing and drying of the material, was 78%.

*Example 5*

A layer of 18x12 open-mesh, bleached gauze was lightly pressed to a piece of like area from a header roll of carded bleached cotton weighing 45 grams per square yard and the assembly looped onto a pin frame so as to limit the ultimate shrink to 25% each in the warp and filling directions, or an area shrink of 44%. The combination was then dropped into a tray containing 16% NaOH at -2° C., a diffusion screen placed on top of the sample, and additional caustic solution poured over the screen. The sample was then given a dilute acid wash, a water wash, a suction treatment to remove excess liquids, and dried on a steam can. In the integral final product the yarns were nearly straight, exhibiting only a slight crimp.

*Example 6*

A ply of bleached cotton header roll weighing 60 grams per square yard was lightly pressed to a layer of 44 x 36 cotton gauze of 30's and 40's yarns and the assembly treated in 16% caustic at -2° C. After the integrated sheet material was washed with water, neutralized with dilute acetic acid, rewashed with water and dried on a steam can, an area shrink of the order of 70% was noted.

*Example 7*

Fourteen strands per inch of 30's cotton yarn were positioned between two carded, bleached cotton fiber sheets each weighing 30 grams per square yard and the aggregate treated in 16% caustic at -2° C. The resulting area shrink, after washing and drying of the material, was 80%.

*Example 8*

A layer of bleached cotton header roll weighing 45 grams per square yard and a coextensive piece of 14x7 cotton marquisette of 9's and 4's yarns were lightly pressed together and dropped into a tray containing 16% NaOH at -2° C. After washing and drying processes, similar to those in the above examples, an area shrink of approximately 75% was noted.

*Example 9*

A ply of 80x80 cotton print cloth and a coextensive piece weighing 45 grams per square yard from a header roll of bleached, carded cotton fibers were lightly pressed together and treated with a solution of 16% NaOH at -2° C. After washing and drying, the final area shrink was about 30%.

*Example 10*

At some sacrifice of various desirable characteristics of my products, particularly high integration, one can employ fibers of regenerated cellulose as the spun fiber con-

stituent. However, when employing such fibers, less severe caustic treatment is in order, that is, the solution temperature should be in the range from 15 to 25° C., and the caustic concentration between 16 and 30 percent. If a soft, flexible material is desired, it is advisable to add to the wash predetermined amounts of an inorganic salt soluble in dilute caustic. I have produced a satisfactory product by lightly pressing together a layer of bleached carded cotton header roll and a 20x12 fabric of regenerated cellulose spun by the Viscose process and treating the assembly in a bath of 20% NaOH at 23° C. The material was washed in water containing 10% sodium chloride, rewash in water, and dried. The final area shrink was approximately 55%.

I claim:

1. As an article of manufacture, a unital, coherent, integrated, shrunken textile sheet material having substantial extensibility, conformability, integrity, and resilience and consisting essentially of cotton fibers spun into yarns and in apposition therewith unspun cotton fibers which are chemically swollen, said spun fibers and said unspun fibers being mutually integrated and frictionally interlocked by chemically induced permanent deformations of the said unspun fibers, said deformations being in the form of random kinks, bends, twists, and curls in substantially all three dimensions and being in excess of the deformations normally present in cotton fibers, the unspun fibers being entangled with themselves and with each other and with the spun fibers to which they are in apposition, the entanglement being substantially continuous and uniform throughout the sheet.

2. As an article of manufacture, a sheet material according to claim 1 in which the yarns are arranged in the form of an open-mesh woven fabric.

3. As an article of manufacture, a sheet material according to claim 1 in which the yarns are arranged in the form of an open-mesh, knitted fabric.

4. As an article of manufacture, a sheet material as defined in claim 1 having an extensibility of at least 25% in one direction without appreciable loss of integrity.

5. As an article of manufacture, a unital, coherent, integrated, shrunken textile sheet material having substantial extensibility, conformability, integrity, and resilience and consisting essentially of cotton fibers spun into yarns and in apposition therewith unspun cotton fibers which are chemically swollen, said spun fibers and said unspun fibers being mutually integrated and frictionally interlocked by chemically induced permanent deformations of the said unspun fibers and spun fibers, said deformations being in the form of random kinks, bends, twists, and curls in substantially all three dimensions and being in excess of the deformations normally present in cotton fibers, the unspun fibers being entangled with themselves and with each other and with the spun fibers to which they are in apposition, the entanglement being substantially continuous and uniform throughout the sheet.

15

20

References Cited in the file of this patent

UNITED STATES PATENTS

|           |                |               |
|-----------|----------------|---------------|
| 164,626   | Whipple        | June 15, 1875 |
| 1,058,827 | Wiesner        | Apr. 15, 1913 |
| 1,334,744 | Farr           | Mar. 23, 1920 |
| 1,629,923 | McDermott      | May 24, 1927  |
| 1,722,764 | Rasch          | July 30, 1929 |
| 1,862,208 | Ahnert         | June 7, 1932  |
| 1,980,498 | Nitsche        | Nov. 13, 1934 |
| 2,113,122 | Reed           | Apr. 5, 1938  |
| 2,341,620 | Jackson et al. | Feb. 15, 1944 |
| 2,370,365 | Magill         | Feb. 27, 1945 |

FOREIGN PATENTS

|               |         |
|---------------|---------|
| Great Britain | of 1903 |
|---------------|---------|